

United Sta

O'Brien

[11] 3,816,212

[45] June 11, 1974

## SUBSTITUTE FOR MISSING XR

[54] PROCESS FOR BONDING AND FLAME PROOFING WEBS OF SYNTHETIC FIBERS

[75] Inventor: Samuel James O'Brien, Dunnellen, N.J.

[73] Assignee: American Cyanamid Company, Stamford, Conn.

[22] Filed: Nov. 13, 1970

[21] Appl. No.: 89,531

[52] U.S. Cl. .... 156/331, 106/15 FP, 117/136, 117/137, 117/138.8 F, 117/138.8 N, 117/138.8 UA, 161/403, 260/29.4, 260/DIG.

24

[51] Int. Cl. .... C09j 5/06, B44d 1/46, B44d 1/09

[58] Field of Search..... 156/331; 106/15 FP; 252/8.1; 117/136, 137

## [56] References Cited

## UNITED STATES PATENTS

2,488,034 11/1949 Pingree et al. .... 117/136

|           |         |                        |           |
|-----------|---------|------------------------|-----------|
| 2,781,281 | 2/1957  | Berger .....           | 117/136   |
| 2,953,480 | 9/1960  | Burnell .....          | 117/137   |
| 3,047,425 | 7/1962  | Hirshfield et al. .... | 117/136 X |
| 3,253,881 | 5/1966  | Donahue.....           | 117/137 X |
| 3,479,211 | 11/1969 | Goldstein.....         | 117/136   |
| 3,496,155 | 2/1970  | O'Connor et al. ....   | 8/192     |

Primary Examiner—George F. Lesmes

Assistant Examiner—J. Cannon

Attorney, Agent, or Firm—Charles Joseph Fickey

[57]

## ABSTRACT

Method for forming a bonded and flame retardant non-woven web of synthetic fibers by treating a web of non-woven synthetic fibers with a thermosetting aminoplast resin, cyanamide and phosphoric acid, and thereafter heating said web at an elevated temperature.

6 Claims, No Drawings

N P

## PROCESS FOR BONDING AND FLAME PROOFING WEBS OF SYNTHETIC FIBERS

The invention relates to a method for forming a bonded and flame retardant nonwoven web of synthetic fibers.

Nonwoven webs of synthetic fibers, particularly polyester fibers such as Dacron, are used as interliners in quilted outer garments. Such webs are made, as well known in the art, by random orientation of synthetic fibers in layers in any desired quantity, depending on the density and thickness desired in the final treated web. In view of the current interest, especially the emphasis by the various governmental bodies, in flame retardant textile materials for wearing apparel, there is a need for flame resistant nonwoven interliners for garments.

A method has now been discovered for producing a bonded and flame retardant nonwoven web of synthetic fibers. By the process of this invention a nonwoven web of synthetic fibers is treated with a thermosetting aminoplast resin, cyanamide and phosphoric acid, and the web is heated at an elevated temperature.

Conventional nonwoven webs of synthetic fibers such as polyester, polyamide and acrylic fibers may be employed.

The thermosetting aminoplast resins of use in this invention are of the conventional types, and include melamine-formaldehyde condensates, urea-formaldehyde condensates, uron-formaldehyde condensates, triazole-formaldehyde condensates, etc. The methylolated products can be alkylated by reaction with lower alcohols, also according to conventional procedures. The preferred resins are methylolated polymethylol melamines.

The resin, cyanamide and phosphoric acid can be applied simultaneously or separately to the web. Solutions of the agents in water or other inert solvent are conveniently applied by padding, spraying or dipping.

The amount of aminoplast resin applied to the web should be between 5 percent and 25 percent, preferably between 7.0 percent and 15.0 percent, based on the weight of the web.

The amount of cyanamide applied to the web should be between 2 percent and 20 percent, preferably between 5 percent and 10 percent, based on the weight of the web.

The amount of phosphoric acid applied to the web should be between 1 percent and 5 percent, preferably between 2 percent and 3 percent, based on the weight of the web.

The treated webs are dried to remove the water or other solvent and are then heated at a temperature between 130° and 180°C., preferably between 149° and 163°C., to effect a cure of the aminoplast resin. If desired, the thickness of the web can be maintained mechanically during the curing step.

### EXAMPLE 1

A pad bath containing 7.2 percent of a partially methylolated trimethylolmelamine, 5 percent of cyanamide and 3.3 percent of 85 percent orthophosphoric acid was applied to a loose web of polyester (Dacron brand) fibers by a standard padding procedure. A wet pickup of 300 percent based on the weight of the web was obtained. The treated loose web was dried for five minutes at 105°C., and the web was then clamped to a

thickness of 0.25 inch and heated at 160°C. for five minutes. The resulting bonded polyester web had a thickness of 0.25 inch and its flame retardancy was commercially acceptable.

### EXAMPLE 2

A loose web of acrylic fiber was treated in a pad bath containing 10 percent of partially methylolated trimethylolmelamine, 8 percent cyanamide and 2 percent of 85 percent orthophosphoric acid, to obtain a wet pickup of about 250 percent. The treated web was dried for about five minutes at 100°C. and then clamped to a thickness of 0.25 inch and heated at 150°C. for five minutes. The resulting acrylic web had a final thickness of about 0.25 inch and commercially acceptable flame retardancy.

### EXAMPLE 3

A polyamide web (Nylon) was treated as in Example 1, with similar results.

### EXAMPLE 4

When the procedure of Example 1 was repeated with substitution of an equal amount of dimethylol 4,5-dihydroxydiethyleneurea for the partially methylolated trimethylol melamine, essentially the same results were obtained.

### EXAMPLE 5

When the procedure of Example 1 was repeated with substitution of an equal amount of dimethylolmelamine for the partially methylolated trimethylolmelamine, essentially the same results were obtained.

### EXAMPLE 6

When the procedure of Example 1 was repeated with substitution of an equal amount of dimethyloleurea for the partially methylolated trimethylol melamine, the resulting polyester web had a high degree of flame retardancy.

I claim:

1. A method for forming a bonded and flame retardant nonwoven web of synthetic fibers comprising impregnating the web with an aqueous solution of a thermosetting aminoplast resin, cyanamide and phosphoric acid and heating the web to effect a cure of the finish on the web.

2. A method as in claim 1 where the synthetic fiber is a polyester fiber and the thermosetting aminoplast resin is a melamine-formaldehyde condensation product.

3. A method as in claim 1 wherein the amount of aminoplast resin is from about 5 to 25 percent based on the weight of the web.

4. A method as in claim 1 wherein the amount of cyanamide is from about 2 to 20 percent based on the weight of the web.

5. A method as in claim 1 wherein the amount of phosphoric acid is from about 1 to 5 percent based on the weight of the web.

6. A method for forming a bonded and flame retardant nonwoven web of synthetic fibers comprising impregnating the web with an aqueous solution of a thermosetting aminoplast resin, cyanamide and phosphoric acid and heating the web to effect a cure of the finish on the web, said heating being at a temperature of about 130° to 180°C.

\* \* \* \* \*